

1,393,355.

J. C. EMHARDT.  
COATED ARTICLE.  
APPLICATION FILED FEB. 25, 1918.

Patented Oct. 11, 1921.



Inventor  
John Charles Emhardt  
By his Attorneys  
Brindle, Wright and Small.

# UNITED STATES PATENT OFFICE.

JOHN CHARLES EMHARDT, OF WILMINGTON, DELAWARE, ASSIGNOR TO E. I. DU PONT DE NEMOURS & COMPANY, OF WILMINGTON, DELAWARE, A CORPORATION OF DELAWARE.

## COATED ARTICLE.

1,393,355.

Specification of Letters Patent. Patented Oct. 11, 1921.

Application filed February 25, 1918. Serial No. 219,091.

To all whom it may concern:

Be it known that I, JOHN CHARLES EMHARDT, of Wilmington, in the county of New Castle, and in the State of Delaware, have

5 invented a certain new and useful Improvement in Coated Articles; and I do hereby declare that the following is a full, clear, and exact description thereof.

My invention relates particularly to fire-  
10 protective coatings, especially such coatings which are comprised of an under coating containing a cellulose ester and an upper coating containing a fire-resisting paint.

The object of my invention is to provide  
15 coatings for surfaces of various kinds which provide an extremely effective protection against ignition and spread of fire.

The object of my invention is to provide compositions of the above character which  
20 will effectively withstand ignition under the conditions to which they are subjected in actual practice.

A further object is to provide compositions of this character which are especially  
25 applicable for use in coating airplanes.

Particularly the object of my invention is to provide compositions of this nature which will prevent ignition of the airplane surfaces beneath coatings of such compositions,  
30 as for example when gasoline or other inflammable liquids are dropped upon the coated surfaces and ignited thereon. That is to say, the object of my invention is to provide such coating compositions which  
35 will protect the airplanes coated thereby from ignition by a larger quantity of burning gasoline on the coated surfaces than surfaces coated with previous coating compositions would withstand.

40 A further object is to provide compositions of this nature which are waterproof, have a low resistance to the air, and which provide the necessary strength and shrinkage after application but without danger of  
45 cracking in use.

Still another object of my invention is to provide fireproof substances for use in compositions of this character which will give off fire suppressing gases, as for example  
50 ammonia or water, as in the case of the water of crystallization, or water of con-

stitution, under the influence of heat, so as to form a protective blanket thereby to retard combustion and prevent the spread of fire.

55

Another object is to provide fireproofing substances of this kind which provide a liquid blanket or absorb heat due to physical or chemical changes therein when heated.

A further object is to utilize substances  
60 of this character which have a low solubility in water.

More particularly the object of my invention is to provide protective coatings of the above character comprising a lower coating  
65 containing a cellulose ester, as for example nitrocellulose or cellulose acetate, with or without the presence of fire-retarding constituents, and an upper coating of a drying oil containing fire-retarding constituents.

70

Further objects of my invention will appear from the detailed description thereof contained hereinafter.

While my invention is capable of being carried out in many different ways, for the  
75 purpose of illustration I shall describe only certain forms of my invention hereinafter.

For example, I may use one of many different fire-proofing constituents for the  
80 nitrocellulose compositions of the kind hereinabove referred to, but among those which I prefer for this purpose are:

Ammonium magnesium phosphate,

$\text{NH}_4\text{MgPO}_4 \cdot 6\text{H}_2\text{O}$ ,

85

Ammonium phosphate,  $\text{H}_2\text{NH}_4\text{PO}_4$ ,

Ammonium magnesium arsenate,

$\text{MgNH}_4\text{AsO}_4 \cdot 6\text{H}_2\text{O}$ ,

Ammonium manganese phosphate,

$\text{NH}_4\text{MnPO}_4 \cdot \text{H}_2\text{O}$ ,

90

Ammonium manganese arsenate,

$\text{MnNH}_4\text{AsO}_4 \cdot 6\text{H}_2\text{O}$ .

Other ammonium salts may be used for this purpose, if desired, or other salts adapted to give off such protective gases or  
95 liquids.

A coating composition which may be made in accordance with my invention and which is particularly adapted for coating the cloth covering airplanes may be the following:

100

For example, the lower coating may be comprised of an ordinary cellulose ester

coating composition, such as a pyroxylin composition, which may contain:

7% by weight of pyroxylin,  
63% by weight of acetone,

5 30% by weight of amyl acetate.

Or, instead, I may use any composition of this general nature containing a fire-retarding constituent.

I may use one of many different fireproofing constituents for the nitrocellulose coatings of the kind hereinabove referred to.

A fireproof coating which may be made in accordance with my invention and which is particularly adapted for coating the cloth 15 covering airplanes may be the following:

7% by weight pyroxylin,

7% by weight ammonium magnesium phosphate,

56% by weight acetone,

20 30% by weight amyl acetate.

The surface to be coated, as for example, the surface of an airplane, may be provided with several coats of one of the above compositions. In the above compositions, I 25 may substitute cellulose acetate for the pyroxylin, if desired. In any of the foregoing compositions I may use 30% by weight of a diluent such as benzol, toluol or benzine, if desired.

30 Thereafter I may apply one or more coats of a fire-retarding paint, that is to say, an oil coating composition containing fire-retarding constituents, of which the following may be an example:

35 35% by weight boiled linseed oil,

25% by weight ammonium magnesium phosphate,

1% by weight of a drier, such for example as cobalt linoleate,

40 29½% by weight of turpentine or turpentine substitute.

Other drying oils may be used instead of the linseed oil, if desired.

The proportions in any or all of the above 45 compositions may be varied within wide limits. The ammonium magnesium phosphate is insoluble in water and when heated gives off ammonia and water of crystallization and water of constitution. The am-

50 monia and water of crystallization and constitution provide smothering gases. The water acts also as a liquid blanket and absorbs heat due to the physical and chemical change in liberating the water of crystallization and constitution.

55 The liberation of the water of crystallization and constitution absorbs heat and the vaporization of the water thus liberated results also in the absorption of heat. In the accompanying drawings,

Figure 1 is a perspective view of a portion of the article embodying my invention;

Fig. 2 is an enlarged sectional view of a portion of the article with the cellulose ester 65 coating applied;

Fig. 3 is a similar view of the completed article.

As appears from the legends on the drawing, the fabric 1, or other surface which is to be coated, is first given a coating 2 of 70 a cellulose ester, and thereafter a coating 3 of a fire-retarding paint is applied and the solvents allowed to evaporate.

Any further additional constituents of any desired character may be added, if desired, to the above compositions. Various solvent mixtures may be used, as for example, solvents including ethyl acetate, methyl acetate and ethyl alcohol as the solvent constituents, and benzol, toluol, and 80 benzine as diluents. For example, I may add thereto 30% by weight of any of the above mentioned diluents. Also I may add any proportion of pigments, and oils as in the following examples:

85 6% by weight pyroxylin,

1% by weight color pigment, such as zinc oxid,

6% by weight ammonium magnesium phosphate.

90 1% by weight castor oil,

56½% by weight acetone,

30% by weight amyl acetate,

or

15½% by weight boiled linseed oil,

15½% by weight poppy oil,

31% by weight ammonium magnesium phosphate.

100 ½% by weight of a drier, such as cobalt linoleate,

3% by weight color pigment, such as zinc oxid,

34½% by weight of turpentine or turpentine substitute.

In order to provide compositions giving 105 off other protective gases than ammonia, I may substitute for the ammonium compounds in the above compositions magnesium carbonate or calcium carbonate which give off carbon dioxide under the influence of heat. Furthermore, ammonium phosphate, which is above referred to, when used, not only gives off ammonia and water of constitution, but provides a liquid blanket of phosphoric acid which retards the fire. 110

While I have described my invention above in detail, I wish it to be understood that many changes may be made therein without departing from the spirit of the invention.

115 I claim:

1. An article having a coating comprising a layer of a cellulose ester coating composition and a covering layer of a composition containing a substance which will give off 125 a fire-retarding gas when heated.

2. An article having a coating comprising a layer of a cellulose ester coating composition and a covering layer of a composition containing a drying oil and a substance 130

which will give off a fire-retarding gas when heated.

3. An article having a coating comprising a layer of a cellulose ester coating composition containing a fire-retarding substance, and a covering layer of a composition containing a substance which will give off a fire-retarding gas when heated.

4. An article having a coating comprising a layer of a cellulose ester coating composition containing a fire-retarding substance, and a covering layer of a composition containing a drying oil and a substance which will give off a fire-retarding gas when heated.

5. An article having a coating comprising a layer of a cellulose ester coating composition containing a substance which will give off a fire-retarding gas when heated, and a covering layer of a paint containing a drying oil and a fire-retarding substance.

6. An article having a coating comprising a layer of a cellulose ester coating composition containing ammonium magnesium phosphate, and a covering layer of a composition containing a drying oil and ammonium magnesium phosphate.

7. An article having a coating comprising a layer of a cellulose ester coating composition, and a covering layer of a composition containing ammonium magnesium phosphate.

8. An article having a coating comprising a layer of a cellulose ester coating composition, and a covering layer of a composition containing a drying oil and ammonium magnesium phosphate.

9. An article having a coating comprising a layer of a cellulose ester coating composition, and a covering layer of a composition

containing a pigment and a fire-retarding substance.

10. An article having a coating comprising a layer of a cellulose ester coating composition, and a covering layer of a composition containing a pigment and a substance which will absorb heat by chemical change when subjected to heat or fire.

11. An article having a coating comprising a layer of a cellulose ester coating composition, and a covering layer of a composition containing a substance which will absorb heat by chemical change when subjected to heat or fire.

12. An article having a coating comprising a layer of a cellulose ester coating composition containing a solvent therefor, and a covering layer of a composition containing a drying oil and ammonium magnesium phosphate.

13. An article having a coating comprising a layer of a cellulose ester coating composition containing a solvent therefor and ammonium magnesium phosphate, and a covering layer of a composition containing a drying oil and ammonium magnesium phosphate.

14. An article having a coating comprising a layer of a cellulose ester coating composition containing a solvent therefor and ammonium magnesium phosphate, and a covering layer of a composition containing a drying oil, a drier, ammonium magnesium phosphate, and turpentine.

In testimony that I claim the foregoing I have hereunto set my hand.

JOHN CHARLES EMHARDT.

Witnesses:

STANLEY L. ABRAMS,  
G. D. HOPKINS.